

Aug. 10, 1965

T. T. KASHIWABARA

3,199,982

DIAZOTYPE REPRODUCTION MATERIAL

Filed March 19, 1963

FIG. 1



FIG. 2



FIG. 3



INVENTOR  
THOMAS KASHIWABARA

BY

*J. Russell Jr. Jr.*

ATTORNEY

1

3,199,982

DIAZOTYPE REPRODUCTION MATERIAL  
Thomas T. Kashiwabara, Fort Lee, N.J., assignor to  
Keuffel & Esser Company, Hoboken, N.J., a corporation of New Jersey

Filed Mar. 19, 1963, Ser. No. 266,332

20 Claims. (Cl. 96—49)

This invention relates to diazotype reproduction materials and methods for their production and use, and refers more particularly to two-component photosensitive diazotype reproduction materials which are developable by means of heat, and to the methods and means for accomplishing the heat development of said materials.

Photosensitive diazotype materials are well known and have many advantages over other means of reproduction when considering the combined basis of quality and cost. The photosensitive diazotype materials, however, possess some inherent disadvantages depending upon their type.

There are two general types of photosensitive diazo systems and materials based on the means of development: the two-component diazotype materials using the dry method of diazo development; and the one-component diazotype materials using the semi-wet method of diazo development.

The dry diazo materials utilize gaseous ammonia to raise the pH of the coating after exposure to allow coupling of the diazo compound and coupler which are coated on the same support. The obvious disadvantage of this system is that it requires the use of gaseous ammonia which is obnoxious and dangerous to handle, and which requires exhaust equipment in order to be utilized in confined spaces.

The semi-wet system of diazo development utilizes a photosensitive material which comprises a base sheet and a coating of photosensitive diazo compound coated on the base sheet. After exposure under a master to actinic light, the sheet coated with the diazo compound is passed through a chemical bath which contains an alkali and a coupler to develop the image by dye formation. Among the major disadvantages of this method is that a liquid is required in the development step. The liquid affects the paper base and requires drying.

Among the old attempts at producing a heat-developable reproduction material was one which utilized a base sheet having a dark background on which a layer of a light-colored wax was applied. The master was placed against the wax layer and was exposed to infra-red radiation which was converted in the image areas to heat which then passed by conduction to the wax layer. The wax layer melted under those portions of the master which contained an image and allowed the dark background of the base sheet to be seen, which in effect reproduced the master image. The disadvantages of this system of reproduction were cost as compared to the conventional diazo systems, quality inferior to the diazo product, and retained heat sensitivity.

The old systems used melting wax layers and the like in heat sensitive and not necessarily light sensitive materials.

For many years heat development of photosensitive diazo materials had been tried without noteworthy success. It had been attempted in order to eliminate the disadvantages of gaseous ammonia in the dry developing system, and liquid developer in the semi-wet system.

The development of exposed two-component diazotype prints by gases given off by the decomposition of ammonia compounds from a developing sheet under the influence of heat had been tried. The ammonia compounds found to be particularly suitable for development of diazotype prints were the products of ammonia and weak acids. Good results were obtained from ammonium carbonate,

2

ammonium bicarbonate, and the like, which decompose freely at temperatures slightly above room temperature with the release of free gaseous ammonia and water vapor. The solid carbonates were heated in juxtaposition to the exposed two-component diazotype paper to fully utilize the released gaseous ammonia on the exposed surface. This known material had the great disadvantage of very poor shelf life which severely limited its practical use.

Another known material incorporated urea with a photosensitive diazoic. The urea decomposed with the heat and liberated ammonia gas which neutralized and acid formed during coupling thereby aiding the coupling of the diazoic with its photolysis phenol. Urea in a separate stratum was tried in another material.

Developing sheets impregnated with a composition containing one compound or a combination of compounds which liberated the vapor of an alkali or a coupler were also tried. Another material incorporated a carboxamide such as formamide, acetamide, urea, and methyl-urea as a humectant but not as a source of alkali ammonia.

Another material was a multilayer diazotype material comprising a support, a layer containing a diazo compound, a fusible barrier layer which melted below the decomposition temperature of the diazo compound, and a layer containing a coupler, all coated on one side of a support. The diazotype material was placed in contact with a master and subjected to infrared radiation. Image-wise generation and transfer of heat from the master to the multilayer diazotype material melted the fusible barrier layer and permitted the diazo compound and coupler to form an azo dye.

Therefore, one object of the present invention is to provide a photosensitive heat developable diazotype material, method, and system which overcomes the disadvantages of prior art.

Another object is to provide a photosensitive heat-developable diazotype material and system which requires neither gaseous ammonia nor liquid developer for development.

Another object is to provide a photosensitive two-component heat-developable diazotype reproduction material which is heat-developable and which is stable to further application of heat.

Another object of the present invention is to provide a photosensitive heat-developable diazotype material which is inexpensive and which gives good quality diazo reproduction.

Other objects will be apparent from the following specification.

In the present invention, the base necessary for the development is produced on the diazotype material at the time of development by thermally induced chemical or physical conversion of a base-releasing compound.

The application of heat causes this compound to release the base necessary for the coupling reaction at the time of development.

It has been found that many organic nitrogen compounds are suitable sources of base for heat-developable diazo materials. These compounds can be incorporated in a sensitizing layer, in a precoat layer, or in a developing sheet depending upon solubility and compatibility. The compounds of the present invention are induced by elevated temperatures to release a base which increases the alkalinity of the system and permits coupling to take place, thereby developing the latent image.

The organic nitrogen compounds suitable for use in the present invention are those corresponding to the following general formula and salts thereof:

70  $R_1NHR_2$   
wherein  $R_1$  and  $R_2$  are members selected from the groups

consisting of: group A where  $R_1$  is a member selected from the group consisting of alkyl, hydroxyalkyl, ethoxy-carbonyl alkyl, carboxyalkyl, carboxy carbamoyl alkyl, guanyl, arylguanyl, aminoguanyl, diallylaminotriazinyl, arylamino triazinyl, thiazolyl, and pyridyl, and  $R_2$  is a member selected from the group consisting of hydrogen, alkyl, and guanyl; and group B when  $R_1$  and  $R_2$  are members of the same heterocyclic ring.

One sub-generic group of chemicals is that corresponding to the general formula and salts thereof:



where  $R_1$  is a member selected from the group consisting of alkyl, hydroxyalkyl, ethoxycarbonylalkyl, carboxy-alkyl, carboxycarbamoyl alkyl, guanyl, aryl-guanyl, aminoguanyl, diallylaminotriazinyl, arylamino triazinyl, thiazolyl, and pyridyl, and  $R_2$  is a member selected from the group consisting of hydrogen, alkyl, and guanyl.

This group includes n-butylamine (as HCl salt), dodecylamine, tetradecylamine, hexadecylamine, octadecylamine, N-methyl glucamine, glycine ethyl ester (as HCl salt), alpha-alanine, L-glutamine, guanidine (as the acetate salt), aminoguanidine (as the sulfate salt), amino-guanidine (as the bicarbonate salt), phenyl guanidine (as the carbonate salt), phenyl biguanide, N, N-diallylmelamine, 2,4-diamino-6-phenyl-s-triazine, 2-aminothiazole, and 2-aminopyridine.

Another sub-generic group is that corresponding to the following general formula:



wherein  $R_1$  and  $R_2$  are members of the same heterocyclic ring. This group includes imidazole, benzimidazole, and piperazine (as the hexahydrate).

In the drawings:

FIGURE 1 is a sectional view of a heat-developable two-component photosensitive diazotype reproduction material 10 comprising a support 11 and a heat-developable two-component photosensitive diazotype layer 12 coated on said support;

FIGURE 2 is a sectional view of a heat-developable two-component photosensitive diazotype reproduction material 20 comprising a support 21, a precoat layer 22 coated on said support, and a two-component photosensitive diazotype layer 23 coated over said precoat layer on said support; and

FIGURE 3 is a sectional view of a developing sheet 30 comprising a support 31 and a heat-activatable developing agent 32 impregnated in said support. The developing sheet is in contact with a two-component photosensitive diazotype reproduction material 40 comprising a support 41 and a two-component photosensitive diazotype layer 42 coated on said support.

One method of the present invention for the preparation of a heat-developing reproduction material is to treat a support material with a solution of heat-activatable developing agent. After drying, the same support is coated on the same side or on the opposite side with a sensitizing solution comprising diazonium compound and coupler. The coating is dried. In this method the heat-activatable developing agent is in the first or precoat layer. The sensitized support is exposed through a master to actinic radiations and is then developed by heat in the range between the activation temperature of the developing agent and the scorching temperature of the support material. The heat-activated liberation of developing agent then causes the image to develop. The preparation and use of heat-developable two-component photosensitive diazotype reproduction material precoated with heat-activatable developing agent of the present invention is illustrated in Example 5.

In another method of preparation of the present invention, the heat-activatable developing agent is incorpo-

rated into the sensitizing with the photosensitive solution comprising diazonium compound and coupler. The solution is applied to a support and then dried. The sensitized support is exposed through a master to actinic radiations and after exposure, heat is applied to the support. The temperature is preferably in range between the activation temperature of the developing agent and the scorching temperature of the support material. This method of preparation is illustrated in Example 3.

A developing sheet is prepared by impregnating a support with a solution of heat-activatable developing agent in a suitable solvent. The solvent is then removed by drying. The developing sheet is used to develop an exposed two-component photosensitive diazotype reproduction material by placing it in face-to-face contact with the exposed sensitized surface of the diazotype material and subjecting the assembly to heat in the range between the activation temperature of the developing agent and the scorching temperature of the diazotype support. This activates the developing agent and permits coupling to occur on the sensitized surface of the diazotype material. The preparation and use of a developing sheet utilizing the heat-activatable developing agent of the present invention is illustrated in Example 1.

The developing temperature range is determined by two factors: first, the activation temperature of the heat-activatable developing agent; and second, the scorching temperature of the diazotype support material. The activation temperature is that degree of heat necessary to release or liberate the developing agent in the amount required for development of a two-component photosensitive diazotype reproduction material. The scorching temperature is that degree of heat which darkens the background of a developed diazotype print or which causes undesirable physical degradation of the diazotype support material.

The examples herein are given for purposes of illustration, and it is to be understood that the invention is not limited to these examples.

40

## EXAMPLES

*Example 1.*—A developing sheet was prepared by impregnating a porous support with a solution and drying the support to remove the solvent. The following formula was used:

|              | G. |
|--------------|----|
| Ethanol      | 90 |
| Dodecylamine | 10 |

The prepared developing sheet was used to heat-developing sheet was used to heat-develop a diazotype reproduction material by placing it in contact with the sensitized surface of the reproduction material that had been exposed to actinic radiations through a master; heating the developing sheet for a few seconds at 150° C. while in contact with the sensitized surface of the reproduction material to release the base and thus effect coupling, and finally, separating the developing sheet from the diazotype reproduction material. A colored dye image was formed on the diazotype reproduction material.

Tetradecylamine, hexadecylamine, octadecylamine, 2-amino-thiazole, 2-aminopyridine, and benzimidazole were used in place of the dodecylamine to produce the same result.

*Example 2.*—N-methyl glucamine was used from a 10% aqueous solution to prepare a developing sheet as in Example 1. Used in the same manner to heat-develop a diazotype reproduction material, the same results were obtained.

Piperazine hydrate was also used from aqueous solution in the same strength to produce the same results.

75

Example 3.—N-methyl glucamine was used as a sensitizing solution according to the following formula:

|                                                                | G.   |
|----------------------------------------------------------------|------|
| Water                                                          | 150  |
| Tartaric acid                                                  | 1/2  |
| Trichloroacetic acid                                           | 7    |
| 1,3,6-naphthalenetrisulfonic acid, sodium salt                 | 6    |
| N-methyl glucamine                                             | 5    |
| p-Dimethylamino benzene diazonium chloride, zinc chloride salt | 4 10 |
| 2,3-dihydroxy-naphthalene-6-sulfonic acid, sodium salt         | 5    |
| Thiourea                                                       | 7    |
| Zinc chloride                                                  | 4    |

This was coated on a support and dried. After exposure to actinic radiations through a master, the sensitized support was heated at a temperature between the melting point of the N-methyl glucamine and the scorching temperature of the support. A blue image corresponding to the master image was produced.

Imidazole, n-butylamine hydrochloride, L-glutamine, glycine ethyl ester hydrochloride, phenyl biguanide, aminoguanidine sulfate, guanidine acetate, and phenyl guanidine carbonate were used in place of N-methyl glucamine. Aminoguanidine bicarbonate was used in half quantities. All produced a blue image with the exception of aminoguanidine sulfate which produced a red-violet image.

Example 4.—N,N-diallyl melamine was used in a pre-coat layer coated from the following solution:

|                      |     |     |
|----------------------|-----|-----|
| Dioxane              | ml. | 100 |
| N,N-diallyl melamine | g.  | 20  |

The precoated support was then coated with the following sensitizing solution:

|                                                                | G.   |
|----------------------------------------------------------------|------|
| Water                                                          | 150  |
| Tartaric acid                                                  | 1/2  |
| Trichloroacetic acid                                           | 5    |
| 1,3,6-naphthalenetrisulfonic acid                              | 6    |
| p-Dimethylamino benzene diazonium chloride, zinc chloride salt | 4    |
| 2,3-dihydroxynaphthalene-6-sulfonic acid, sodium salt          | 5 45 |
| Thiourea                                                       | 7    |
| Zinc chloride                                                  | 4    |

After the sensitized support was dried, it was exposed to actinic radiations through a master and then heat-developed for a few seconds at 150° C. to produce a blue image corresponding to the master image.

Example 5.—2,4-diamino-6-phenyl-s-triazine was used from a saturated solution in dioxane to prepare a pre-coat layer on a support. This was then sensitized as in Example 4 to produce substantially the same results when heat-developed.

Example 6.—The sensitizing solution of Example 3 was prepared with 3 g. of benzimidazole in place of 5 g. of N-methyl glucamine. After a support was sensitized and heat-developed as in Example 3, a blue image corresponding to the master image was produced.

Example 7.—A mixture of the following composition was used to prepare a developing sheet:

|                                                               | Percent |
|---------------------------------------------------------------|---------|
| Tetradecylamine acetate                                       | 5       |
| Hexadecylamine acetate                                        | 30      |
| Octadecylamine acetate                                        | 65      |
| The solution was prepared according to the following formula: |         |
| Ethanol                                                       | 95      |
| Amine acetate mixture                                         | 5       |

A support was impregnated with this solution and then dried to produce a developing sheet. This was used to heat-develop a diazotype reproduction material as in Example 1 to produce a dye image corresponding to the master image.

Example 8.—A sensitizing solution was prepared according to the formula in Example 3 using 15 g. alpha-alanine in place of the 5 g. N-methyl glucamine. The solution was coated on a support and heat-developed to produce a blue dye image corresponding to the master image.

It is apparent that the described examples are capable of many variations and modifications within the scope of the present invention. All such variations and modifications are to be included within the scope of the present invention.

What I claim is:

1. A heat-developable diazo-type material, which comprises:  
a support resistant to the scorching effects of heat at the conditions of thermal development; and  
a photosensitive diazonium compound, a coupler therefor, and a heat-activatable developing agent coated on said support, said agent having the general formula:



where  $R_1$  and  $R_2$  are members selected from one of the groups consisting of:

group A in which  $R_1$  is a member selected from the group consisting of: alkyl, thiazolyl, pyridyl, guanyl, and triazinyl, and  $R_2$  is a member selected from the group consisting of hydrogen, methyl, and guanyl; and

group B in which  $R_1$  and  $R_2$  are members of the same heterocyclic ring.

2. A method for making a diazo reproduction of an image, which comprises the steps of:  
exposing a diazo sheet to imagewise actinic radiation, said sheet comprising a support resistant to the scorching effects of heat at the conditions of thermal development, and a photosensitive diazonium compound, a coupler therefor, and a heat-activatable developing agent coated on said support, said agent having the general formula:



where  $R_1$  and  $R_2$  are members selected from one of the groups consisting of:

group A in which  $R_1$  is a member selected from the group consisting of alkyl, thiazolyl, pyridyl, guanyl, and triazinyl, and  $R_2$  is selected from the group consisting of hydrogen, methyl, and guanyl; and

group B where  $R_1$  and  $R_2$  are members of the same heterocyclic ring; and

heating said sheet at a temperature between the activation point of said agent and the scorching point of said support to form a dye image on said sheet.

3. A sheet in accordance with claim 1 in which said agent is intimately admixed with said diazo layer.

4. A sheet in accordance with claim 1 in which said agent is coated between said support and said diazo layer.

5. A method in accordance with claim 1 in which said agent is intimately admixed with said diazo layer coated on the same support.

6. A method in accordance with claim 1 in which said agent is coated on said support between said support and said diazo layer.

7. A material in accordance with claim 3 in which said agent is n-butylamine hydrochloride.

8. A material in accordance with claim 3 in which said agent is N-methyl glucamine.

9. A material in accordance with claim 3 in which said agent is phenyl biguanide.

10. A material in accordance with claim 3 in which said agent is guanidine acetate.
11. A material in accordance with claim 3 in which said agent is imidazole.
12. A material in accordance with claim 4 in which said agent is N,N-diallyl melamine.
13. A material in accordance with claim 4 in which said agent is 2,4-diamino-6-phenyl-s-triazine.
14. A method in accordance with claim 5 in which said agent is n-butylamine hydrochloride.
15. A method in accordance with claim 5 in which said agent is N-methyl glucamine.
16. A method in accordance with claim 5 in which said agent is phenyl biguanide.
17. A method in accordance with claim 5 in which said agent is guanidine acetate.
18. A method in accordance with claim 5 in which said agent is imidazole.
19. A method in accordance with claim 6 in which said agent is N,N-diallyl-melamine.
20. A method in accordance with claim 6 in which said agent is 2,4-diamino-6-phenyl-s-triazine.

## References Cited by the Examiner

## UNITED STATES PATENTS

|           |       |                   |            |
|-----------|-------|-------------------|------------|
| 1,807,761 | 6/31  | Sprongerts        | 96—91      |
| 2,459,521 | 1/49  | Greig             | 96—91      |
| 2,545,423 | 3/51  | Duerr             | 96—75      |
| 2,593,911 | 4/52  | Neumann et al.    | 96—91      |
| 2,618,555 | 11/52 | Reichel           | 96—49      |
| 2,668,111 | 2/54  | Lindquist         | 117—154 XR |
| 2,732,299 | 1/56  | Morrison          | 96—49      |
| 2,774,669 | 12/56 | Marron et al.     | 96—49      |
| 2,822,296 | 2/58  | Barrett et al.    | 117—154 XR |
| 3,046,128 | 7/62  | Klimkowski et al. | 96—75 XR   |

## FOREIGN PATENTS

|           |       |                |
|-----------|-------|----------------|
| 816,601   | 7/59  | Great Britain. |
| 1,249,913 | 11/60 | France.        |

## OTHER REFERENCES

Kosar: "Photographic Science & Engineering," vol. 5, No. 4, July-August 1961, pp. 239-243.

NORMAN G. TORCHIN, Primary Examiner.